

# UNITED STATES PATENT OFFICE

2,230,687

## MANUFACTURE OF HIGH SPEED STEELS

Eduard Houdremont and Hans Schrader, Essen, Germany, assignors, by mesne assignments, to Pantena Limited, Glarus, Switzerland, a corporation of Switzerland

No Drawing. Original application February 24, 1938, Serial No. 192,288. Divided and this application March 2, 1940, Serial No. 322,009. In Germany March 31, 1937

2 Claims. (Cl. 75—128)

The present invention relates to steels intended for the manufacture of high speed machining tools, this application being a division of our application Serial No. 192,288. According to the invention such tools are made of steel alloys which contain from 1.0 to 1.6% carbon, from 1.0 to 6.0% chromium, more than 1.0% and less than 5.0% molybdenum, from 2.0 to 6.0% vanadium and up to 5% cobalt, the remainder substantially all being iron with the normal impurities.

Steels of a composition as specified hereinbefore although they contain only small percentages of alloying constituents are distinguished by a high efficiency in the chip-removing working of materials and can be equal in this respect even to the known high alloy high speed tungsten steels or, under favorable cutting conditions, even be superior to them.

The ratio of efficiency to degree of alloying is most favorable with steels according to the in-

vention, which besides iron with the normal impurities contain from 1.2 to 1.5% carbon, from 3.0 to 5.0% chromium, at least 3.0% and less 5.0 molybdenum, from 4.0 to 6.0% vanadium and up to 5% cobalt.

What we claim and desire to secure by Letters Patent is:

1. A high speed steel consisting of 1.0 to 1.6% carbon, 1.0 to 6.0% chromium, more than 1.0% and less than 5.0% molybdenum, 2.0 to 6.0% vanadium and from 0.2 to 5% cobalt, remainder substantially all iron with the normal impurities.

2. A high speed steel consisting of 1.2 to 1.5% carbon, 3.0 to 5.0% chromium, at least 3.0% and less than 5% molybdenum, 4.0 to 6.0% vanadium and from 0.2 to 5% cobalt, remainder substantially all iron with the normal impurities.

EDUARD HOUDREMONT.  
HANS SCHRADER. 20